

Aug. 7, 1934.

E. A. TROEGER

1,969,485

PROJECTION SCREEN

Original Filed Dec. 17, 1926



*Eugene A. Troeger*  
INVENTOR  
BY  
*W.M. J. Cuthand*  
ATTORNEY

## UNITED STATES PATENT OFFICE

1,969,485

## PROJECTION SCREEN

Ernest A. Troeger, Brooklyn, N. Y., assignor, by  
mesne assignments, to Trans-Lux Daylight  
Picture Screen Corporation, New York, N. Y., a  
corporation of Delaware

Application December 17, 1926, Serial No. 155,407  
Renewed May 27, 1932

10 Claims. (Cl. 88—24)

This invention relates to a projection screen of the translucent type in which the image is projected upon the side of the screen opposite to the side which is viewed by the audience. The

5 object of my invention is to provide a screen of that type which may be easily and cheaply made and which will effectively diffuse light striking the screen so as to avoid a glaring bright spot, which is so common with other screens of this 10 nature. Further objects and advantages will appear during the following description of my invention when taken in conjunction with the accompanying drawing, in which

Figure 1 is a diagram showing the use of my 15 screen.

Figure 2 is a cross-sectional view through a portion of the screen.

Many different substances and mixtures have 20 been tried in an effort to obtain a screen which will not only transmit the light from the projector therethrough, but will define a clear-cut image on the side of the screen remote from the projector without the formation of a bright spot of light. I have found that these results may be 25 obtained by forming a screen according to the following method.

For a base I preferably employ a substantially homogenous sheet of wood pulp formed in the following manner. The raw material may 30 be fine wood pulp in any convenient form. It may, for example, be shredded or in the form of saw-dust. This raw material is then digested by being cooked or boiled in a suitable liquid, such as lime or sulphite, and this is best done 35 under steam pressure. The result of this step is a loose, wet, fibrous mass of substantially homogenous material. This mass is then washed in water and bleached in any suitable manner and by any well-known means. The mass is still 40 loose, wet and fibrous in character.

I then add to the above mass a suitable agent as a fine clay or lithopone to act as a diffuser and any desired color may be added at this stage in order to obtain the required 45 shade. The percentage of clay or lithopone will vary according to the amount of diffusion found necessary for the particular screen being built, and the color will vary also and may be omitted altogether if desired.

50 The mass is then rolled out into sheets of the desired thickness and shape and dried. The rollers which are employed for this purpose may be heated if desired in order to facilitate the drying.

55 The sheet formed in this manner is used as a

base for the finished screen and I may apply thereto a coating of translucent diffusing material, this coating being formed in the following manner.

I first make a solution of air-dried soap chips in water, this solution being formed by boiling. I add to this solution a second boiling solution of alum, the two being mixed when boiling or substantially at that temperature. The result of this mixture is a dough-like mass. This mass is then pressed to force out the water and it then easily disintegrates into a fine powder. This powder is then boiled in benzine, forming a liquid which I then apply in a thin film as a coating on one or both sides of the base. It is preferable to coat both sides as the coating is 60 water-resistant and tough and thus protects the base as well as acting as diffuser.

In place of the coating just described above, I may employ another coating made of a mixture of beeswax, linseed oil, gum copal and 65 Venice turpentine. The linseed oil is used to thin out the beeswax and the turpentine thins out the gum copal. The mixture of the two solutions will form a coating which will have 70 the desired characteristics. However, I prefer 75 to form a coating of the material first described above.

In the accompanying drawing I have shown 80 at 1 a suitable projector which is adapted to 85 project an image upon the screen 2, from which it is viewed from the position indicated at 3. The base is indicated at 4 in Fig. 2, and is preferably made in the manner described above. While I have described the base as formed of 90 wood pulp, it is obvious that equivalents of this material may be employed. The essential thing is to have a base of cellulosic material in a translucent form. The base is then supplied with the coatings 5 and 6 on opposite sides thereof, although the coating on one side may be omitted if 95 found desirable.

From the above it will be seen that I have devised a screen for projection purposes and more particularly for so-called rear projection, which 100 may be very cheaply and easily made and which will effectively diffuse light, at the same time forming a sharp, well defined image.

While I have shown one form of my invention I do not intend to limit myself thereto, as I consider myself entitled to all equivalents, and I intend to limit myself only by the appended 105 claims.

I claim:

1. A translucent projection screen comprising 110

- a translucent base formed of wood pulp digested in lime to form a substantially homogenous mass, having a diffusor incorporated therewith, and a coating of translucent diffusing material thereon.
- 5 2. A translucent projection screen comprising a translucent base of wood pulp in a substantially homogenous mass having incorporated therein a fine clay, and a coating on said base formed of a solution of soap and alum in benzine.
- 10 3. A translucent projection screen comprising a base of substantially homogenous translucent cellulosic material having clay incorporated therein, and a coating of translucent diffusing material thereon.
- 15 4. A translucent projection screen comprising a translucent base of wood pulp in a substantially homogenous mass having incorporated therein a fine clay, and a diffusing coating comprising an insoluble soap on said base.
- 20 5. A translucent projection screen comprising a translucent base of wood pulp in a substantially homogenous mass having incorporated therein a fine clay, and a diffusing coating comprising an aluminium soap on said base.
- 25 6. A translucent projection screen comprising a translucent base of substantially homogenous cellulosic material, and a diffusing coating comprising an insoluble soap on said base.
- 30 7. A translucent projection screen comprising a translucent base formed of wood pulp in a substantially homogenous mass and a coating of translucent diffusing material, comprising an aluminium soap on said base.
8. A rear projection screen comprising a translucent base formed principally of substantially homogeneous cellulosic material, a light-diffusing agent substantially uniformly incorporated in said screen base, and a second light-diffusing agent on an exterior surface of said screen, the quantity of said light-diffusing agents being approximately predetermined whereby a substantial amount of light traverses the screen when it is included in a rear projection system. 80
9. A rear projection screen comprising a base formed principally of substantially homogeneous cellulosic material, and light-diffusing means associated with said base to such limited extent that a substantial amount of light traverses the screen when it is included in a rear projection system, said light-diffusing means comprising a light-diffusing agent on an exterior surface of 85 said screen. 90
10. A rear projection screen comprising a base formed principally of substantially homogeneous cellulosic material, and light-diffusing means associated with said base to such limited extent that a substantial amount of light traverses the screen when it is included in a rear projection system, said light-diffusing means comprising a light-diffusing agent substantially uniformly incorporated in and throughout said cellulosic material. 100

ERNEST A. TROEGER.

35

110

40

115

45

120

50

125

55

130

60

135

65

140

70

145

75

150